

## UNITED STATES PATENT OFFICE.

ROBERT MEYER, OF HANNOVER, GERMANY.

## METHOD OF COMBINING LEATHER AND CAOUTCHOUC.

No Drawing. Application filed October 19, 1925, Serial No. 63,543, and in Germany August 1, 1923.

My invention refers to means for combining leather with caoutchouc. It is an object of my invention to produce such combination in a more efficient manner than was hitherto possible.

In combining leather with caoutchouc care has been taken to employ air-dried leather, that is leather dried at the air or in the sun, inasmuch as leather laden with moisture will 10 not enter into an intimate and stable combination with caoutchouc and on being vulcanized will become brittle. It is however well known that the use of air dried leather does not altogether obviate the difficulties 15 encountered in combining these two substances.

In accordance with the present invention the leather, which may be air dried, is subjected to a further drying treatment, preferably by heating it in dry air, for instance in an air dryer during about twenty-four hours to about 50° C. and preventing it from coming in contact with moist air until it is combined with the caoutchouc. To this 20 end the leather thus dried is either stored under the exclusion of air or the combination with caoutchouc is effected immediately after the leather has been withdrawn from the air dryer. In this manner the absorption 25 of moisture can be prevented.

Preferably leather dried according to the present invention is, immediately after the drying operation has come to an end, immersed in a rubber solution, that is a solution of caoutchouc in petrol, whereby the fine pores of the leather are closed so as to prevent the admission of moisture.

In practicing my invention I prefer employing waste leather and preferably the 30 pieces of leather are comminuted by maceration or by grinding, whereupon the dust is removed by sieving and the fibrous or pulv 35 erulent mass is now dried in the manner

above described, whereupon it is mixed with a thinly fluid caoutchouc solution to form a 45 pulp which is then carefully kneaded and dried at an elevated temperature until the material has obtained a satisfactory adhesive power.

With the mass thus obtained plastic products 50 of different kinds can be produced.

Although in consequence of the preheating of the leather a stable combination with caoutchouc can be produced, the stability of 55 the products is increased if they are subjected to vulcanization, preferably after adding sulphur, either in the cold or at an elevated temperature.

If it is for instance intended to treat macerated leather chips, vulcanization at an 60 elevated temperature may be dispensed with, if it is however desired to produce soles, heels or the like for shoes or a floor covering, it is preferable to resort to hot vulcanization inasmuch as the final product thus obtained 65 is more durable than leather. The vulcanization can be effected in such cases at high temperatures inasmuch as there is no danger of the final product getting brittle. For I have ascertained that brittleness is 70 merely caused by a moisture content of the leather.

I wish it to be understood that I do not desire to be limited to the actual sequences 75 of operations, proportions and other details above described for obvious modifications will occur to a person skilled in the art.

I claim:

The method of combining leather and caoutchouc comprising the step of drying 80 the leather for about 24 hours at about 50° C., taking care to prevent access of air to the leather thus dried, and treating same with a solution of caoutchouc.

In testimony whereof I affix my signature.  
ROBERT MEYER.